

April 19, 1927.

1,625,463

E. GAUTHIER

DIAMOND LAP

Filed Dec. 29, 1922



Fig. 3.



Inventor  
Ernest Gauthier  
by Alb. Patterson

Atty.

## UNITED STATES PATENT OFFICE.

ERNEST GAUTHIER, OF CHICAGO, ILLINOIS, ASSIGNOR TO WESTERN ELECTRIC COMPANY, INCORPORATED, OF NEW YORK, N. Y., A CORPORATION OF NEW YORK.

## DIAMOND LAP.

Application filed December 29, 1922. Serial No. 609,645.

This invention relates to improvements in grinding implements and more particularly to diamond laps and to an improved method of making the same.

5 The object of the invention is to produce a diamond lap having superior cutting qualities and long life and provide an inexpensive method of manufacturing the same.

10 Heretofore, laps of this type have been made by forcing diamond powder into the periphery of a metallic arbor, the projecting points of the particles serving as cutters. Laps made in this way are open to the serious objection that the particles become dislodged from their seats in the arbor within 15 a short time and before they have outworn their usefulness. As a result the efficient working life of the lap is of short duration.

15 In accordance with the present invention a 20 grinding implement is produced comprising a suitable arbor and a grinding element composed of abrasive material and a suitable binder molded under pressure to constitute a unitary structure and suitably attached to the arbor. In its preferred form the invention 25 comprises a lap consisting of an arbor and a grinding element composed of diamond splints or particles, and a metallic binder, in powdered form, molded under 30 pressure into a unitary structure, the grinding element thus produced being simultaneously molded onto the arbor.

35 The accompanying drawing illustrates a lap made in accordance with the invention and a method by which the same may be produced, and in which,

40 Fig. 1 is a vertical sectional view, parts shown in the elevation, illustrating an apparatus by which the grinding element may be made and attached to the arbor, and showing a lap in the process of being made thereby;

45 Fig. 2 is a fragmentary top plan view thereof, and,

50 Fig. 3 is a longitudinal sectional view of a completed lap.

55 In making a lap in accordance with the present invention an arbor 10 is set in an upright position within an opening made in a suitable base block 11 to receive it. The arbor 10 may be of any suitable construction, but preferably made of steel and having a portion of its periphery corrugated or fluted in the manner indicated at 12, the purpose of which will be hereinafter de-

scribed. After the arbor has been mounted in position, a mold 13 is fitted within a cup-shaped opening 14 of a size and shape to receive it, made in the base block 11. The mold is provided with a cylindrical opening 15 to receive the material to be molded, this opening communicating with a central orifice through which the fluted end 12 of the arbor 10 projects in the manner shown in Fig. 1. A mixture composed of particles of abrasive material and particles of a suitable binder is then deposited in the opening 15 in the mold. The volume of the mixture placed in the mold may vary in amounts partially or completely filling the opening, according to the size of the grinding element desired. Any suitable abrasive and binding ingredients may be used to constitute the mixture, but in making diamond laps, preferably diamond splints and a binding material consisting of powdered metal is utilized. It will be found that a more uniformly molded grinding element will be produced if a metallic binder is utilized free from impurities, and for this reason preferably electrolytic metal should be used as the binder. I have experienced very satisfactory results using electrolytic iron in a mixture of 66% electrolytic iron and 34% diamond particles. After the abrasive mixture has been placed in the mold, a plunger or ram 16 is caused to descend, the ram being of a size to enter the opening in the mold and having a central opening 17 to receive the projecting end of the arbor 10. The ram 16 may be 70 operated by hydraulic pressure or other suitable means to exert suitable pressure upon the abrasive mixture within the mold.

75 The mixture within the mold is subjected to sufficient pressure by the ram 16 to mold it into a homogeneous aggregate which is interlocked with the ridges and depressions in the fluted end of the arbor so as to be firmly secured thereto.

80 The proportion of the mixture of the diamonds and binder, together with the amount of pressure to be exerted by the ram 16, should vary according to the hardness which it is desired that the molded grinding element should have. I have found that a 85 mixture of 66% electrolytic iron particles and 34% diamond particles molded under pressure of 100 tons per square inch produces a grinding element capable of holding the diamond particles firmly enough for 90 100 105 110

practical grinding purposes, and is not so hard but that it will wear down as the diamond particles become dulled so that they may be wrenched out of their position to expose new diamond particles to the grinding face.

The great efficiency of a lap made in accordance with the present invention as compared with a lap made by forcing diamond 10 splints into a metallic arbor may be made clear by a comparative test of the two laps. Using the old type of lap to lap out a hole in a hardened steel piece, I found that in an hour's time the lap had enlarged the hole 15 by .015. In lapping a similar hole in the same stock with a lap made in accordance with the present invention, I found that in an hour the hole had been enlarged by .049. In other words, I find that when the two 20 laps are used under the same conditions, the lap of the present invention will cut approximately three times as much metal in a given time as the form of lap heretofore used. Furthermore due to the thickness of the 25 grinding implement the improved form of lap has a long working life and the diamond particles are not dislodged from their binder until they have outworn their usefulness.

After the molding operation is completed 30 the ram is raised and the base block 11 inverted. By tapping the end of the arbor

10 with a punch or other suitable device, the completed lap together with the mold 13 will drop out of the base block. The mold 13 is made in three segments and is readily 35 removed by striking it against the base block or giving it a blow with a hammer, which will cause the segments to fall away from the molded grinding element.

What is claimed is:

1. A new article of manufacture comprising diamond particles and finely divided metallic particles molded into a homogeneous aggregate.

2. A new article of manufacture comprising diamond particles and electrolytic metal particles molded under pressure to form a homogeneous aggregate.

3. A new article of manufacture comprising diamond particles and electrolytic iron particles in a finely divided form molded under pressure to form a homogeneous aggregate.

4. A new article of manufacture comprising diamond particles about 66% and electrolytic iron particles about 34 percent molded under pressure to form a homogeneous aggregate.

In witness whereof, I hereunto subscribe my name this 20th day of December, A. D., 60 1922.

ERNEST GAUTHIER.